

Jan. 17, 1956

T. R. YOUNG ET AL.

2,731,405

## METHOD OF PREPARING ELECTROLYTE

Filed Jan. 21, 1953



INVENTORS  
Thomas R. Young  
Robert L. Somerville  
BY

BY  
Pennie, Edwards, Morton, Barrone *and* Taylor  
ATTORNEYS

# United States Patent Office

2,731,405

Patented Jan. 17, 1956

1

2,731,405

## METHOD OF PREPARING ELECTROLYTE

Thomas R. Young, Riverside, Conn., and Robert L. Somerville, Neshanic, N. J., assignors, by mesne assignments, to Horizons Titanium Corporation, Princeton, N. J., a corporation of New Jersey

Application January 21, 1953, Serial No. 332,327

4 Claims. (Cl. 204—64)

This invention relates to the electrolytic production of metallic titanium and metallic zirconium and, more particularly, to a cyclic method wherein spent electrolyte from the titanium or zirconium production stage may be completely recovered and re-used in the electrolytic operation.

The production of metallic titanium and metallic zirconium by electrolytic deposition from a fused salt bath containing an alkali metal-titanium or zirconium double fluoride (an alkali metal fluotitanate or fluozirconate) has been developed to the stage where the metal so produced is of high purity. From a commercial standpoint, however, the cost of producing metal by this procedure is a serious drawback due largely to the cost of raw materials including the fluorine component of the double fluoride. We have now discovered that the cost of raw materials for such a process of electrolytically producing metallic titanium and metallic zirconium can be markedly reduced by appropriate choice of the diluent salt bath and by appropriate conversion of the by-products of the electrolysis. Thus we have found that the completely cyclic handling of all by-products of the electrolysis may be achieved without the build up of any one or more of the elements of the electrolytic bath.

The success of our recyclic operation in the electrolytic production of metallic titanium or metallic zirconium from a fused salt bath is dependent upon the use as the immediate source of the titanium or zirconium of a compound of such metal the anion of which is restricted to one or more of the elements chlorine, oxygen and carbon, by the use as another component of the salt bath of one or more alkali metal chlorides, and advantageously by the use of hydrogen, as the only other extraneous raw material, for conversion of by-product chlorine from the electrolytic cell into hydrogen chloride for use in the transformation of the titaniferous or zirconiferous source material into the corresponding alkali metal double fluoride. Thus, our invention comprises an improvement in the production of metallic titanium or metallic zirconium wherein a double fluoride of titanium or zirconium and an alkali metal is electrolyzed in a fused salt bath comprising this double fluoride dissolved or otherwise contained in an alkali metal chloride, the products of the electrolysis comprising deposited metallic titanium or zirconium, evolved chlorine gas and an alkali metal fluoride-containing spent electrolyte. Our improvement in such a process comprises reacting the spent electrolyte from the aforesaid electrolysis with hydrochloric acid and a titaniferous or zirconiferous source material the anion of which is composed of one or more of the elements chlorine, oxygen and carbon with the resulting formation of an alkali metal-titanium or zirconium double fluoride and an alkali metal chloride which are thereafter used as the double fluoride and alkali metal components of the aforementioned fused salt bath. In the presently preferred embodiment of our invention, the hydrochloric acid is derived by the reaction of chlorine evolved from the electrolytic cell with extraneous hydrogen.

2

The titaniferous sources useful in practicing our invention include oxidic compounds such as titanium dioxide, titanium carbonate and titanium oxychloride ( $TiOCl_2$ ) and titanium carbide. Each of these source materials should be supplied in as pure form as readily available in order to preclude the build up of extraneous impurities in the process. When titanium dioxide is used as the starting material, we have found it advantageous to use anatase titanium dioxide pigment, but other forms of the dioxide may be used with advantage. The oxychloride of titanium as well as the carbonate and carbide are available and can be used as the source of titanium without introducing into the cyclic process any component which will be built up to the detriment of the operation of the process.

The zirconiferous materials useful in practicing our invention include oxidic zirconiferous materials such as zirconium oxides, zirconium carbide and zirconium oxychloride. Thus, inasmuch as the raw materials as well as the chemistry of our process are substantially the same for zirconium as for titanium, we shall confine our subsequent description of the invention to the production of metallic titanium with the understanding, of course, that what is said in this regard applies with equal force to the corresponding production of metallic zirconium.

The only other raw material required in significant amounts for the practice of our invention is hydrogen, and this hydrogen may be supplied either as such or in the form of a mixture of propane and steam which, when burned in the presence of chlorine gas, will yield hydrogen to react with the chlorine to form hydrogen chloride.

The process of our invention will be readily understood by reference to the accompanying flow sheet. As shown therein, an alkali metal-titanium double fluoride, such as potassium titanium fluoride (also known as potassium fluotitanate,  $K_2TiF_6$ ), and at least one alkali metal chloride such as sodium chloride are charged to an electrolytic cell 1 as the essential components of the electrolytic bath. The cell is heated to maintain these salts in fused condition in the cell. Electrolysis of the resulting bath, which may contain, for example, 2 to 30% by weight of the double fluoride, results in the deposition at the cell cathode of metallic titanium which may be removed in any appropriate manner. Chlorine gas is evolved at the anode and is withdrawn from the cell and burned with hydrogen in a combustion chamber 2. The resulting hydrogen chloride is advantageously absorbed in water in an absorption tower 3, and the resulting aqueous hydrochloric acid is delivered to a reactor 4 wherein the alkali metal-titanium double fluoride is produced. Spent electrolyte is withdrawn from the cell either intermittently or continuously, and is delivered to the reactor 4. This spent electrolyte, which contains an alkali metal fluoride as its essential component, may be either cooled and then charged directly to the reactor 4 or it may be broken up into a slurry with extraneous water or other suitable wash liquid from another stage of the process and be delivered in this form to the reactor 4.

The other primary component delivered to the reactor 4 comprises the titaniferous source material such as titanium dioxide or titanium oxychloride. If titanium dioxide is used, it may be charged to the reactor in the form of dry titania pigment. Of course, when the titaniferous material is charged in the form of oxychloride, lesser amounts of hydrochloric acid will be required and any excess acid produced from the cell chlorine may be disposed of or used in any other desirable way. Small amounts of an alkali metal chloride such as potassium chloride and a source of fluorine such as hydrofluoric acid may also be added to the reactor 4 in order to make up for any mechanical loss of the alkali metal, chlorine- and fluorine-components of the fused salt bath and thus insure

the presence in the reactor of substantially stoichiometric quantities of all essential reagents for the formation of an alkali metal-titanium double fluoride.

Inasmuch as the electrolysis of the fused salt bath is preferably carried out under an inert atmosphere, advantageously of a monatomic gas such as argon, the argon will be discharged from the cell along with the chlorine. However, the argon will pass through the combustion chamber 2 and the absorption tower 3 and can thus be returned to the cell 1 preferably with intervening purification to remove any extraneous gas such as nitrogen from leakage or carbon dioxide from the burning of propane, or to remove a gaseous impurity introduced into the system along with the argon.

The reaction between the added titaniferous source material, the generated hydrochloric acid and the recirculated spent electrolyte, together with added make-up reagents, takes place in the reactor 4 upon heating this mixture to a temperature close to the boiling point of water at atmospheric pressure, i. e. up to about 100° C., by means of steam coils or the like. The resulting alkali metal-titanium double fluoride solution, such as a potassium-titanium fluoride solution, is withdrawn from the reactor 4 and is concentrated to crystallize out of the solution both the double fluoride and a portion of the contained alkali metal chloride. We have found that this result can be obtained particularly satisfactorily in a triple effect evaporator, but regardless of the method of separating the double fluoride and the alkali metal chloride these separated salts are passed through driers 5 and 6 and thence back to the electrolytic cell 1. It will be seen, accordingly, that the only extraneous source materials for this continuous production of titanium metal comprises the titaniferous source material, such as titanium dioxide, and hydrogen for the generation of hydrogen chloride from the chlorine effluent from the cell.

As pointed out hereinbefore, we have found that a triple effect evaporator may be used with particular advantage in the recovery of the solid alkali metal-titanium double fluoride and alkali metal chloride from the solution thereof withdrawn from the reactor 4. In the operation of the triple effect evaporator in accordance with our invention, the alkali metal-titanium double fluoride and alkali metal chloride solution (such, for example, as an aqueous solution of potassium titanium fluoride and sodium chloride) is delivered to the third effect of the evaporator. The solution is concentrated in the third effect by the combination of a reduction in pressure, such as operation under a vacuum of say 27 inches of mercury, and by the heat supplied by steam which has previously been used as the heating medium for the first two effects. The liquor in the third effect is thus concentrated at a temperature of about 50° C. with the result that potassium titanium fluoride crystals form in the liquor. The resulting slurry of the double fluoride is discharged from the third effect to a separator 7, and the separated double fluoride is delivered to the drier 5. A portion of the mother liquor removed from the double fluoride in the separator 7 may be returned to the reactor 4 and the remainder of the liquor is delivered to the second effect of the evaporator. Inasmuch as the second effect operates at a higher temperature, generally about 90° C., the further evaporation of water from the liquor introduced into the second effect from the separator 7 results in crystallization of sodium chloride. The resulting slurry is discharged from the second effect to a separator 8 from which the separated sodium chloride is delivered to the drier 6. A portion of the liquor separated from the sodium chloride in the separator 8 is advantageously returned to the third effect and the remainder of this liquor is delivered to the first effect of the evaporator. Inasmuch as the heating steam for the evaporator passes through the first effect before the second and third effects, the temperature of the liquor in the first effect is raised to a still higher temperature, about 130° C. Although a considerable amount of

water is evaporated from the liquor in the first effect, with the resulting crystallization of some sodium chloride, the resulting slurry is delivered to the second effect where further evaporation, though at a lower prevailing operating temperature, effects more complete crystallization of sodium chloride which is then recovered in the separator 8. On the other hand, the potassium titanium fluoride contained in the aqueous phase in both of these relatively high temperature effects will remain in solution and will not crystallize from the solution to any significant extent until it is delivered to the third effect which, as noted hereinbefore, advantageously operates at a relatively low temperature of about 50° C.

The process of our invention may be illustrated by, but 15 is not limited to, the following specific example thereof:

A fused salt bath composed of potassium fluotitanate and sodium chloride, in which the potassium fluotitanate formed 25% of the initial weight of the bath, was electrolyzed in an electrolytic cell maintained under an 20 inert atmosphere of argon gas. For each mol of potassium fluotitanate that was decomposed at the cathode, one mol of titanium was deposited on the cathode, two mols of potassium fluoride were formed, four mols 25 of sodium chloride were converted to four mols of sodium fluoride, and two mols of chlorine gas were evolved from the electrolyte. Chlorine gas evolved from the fused salt bath at the anode and titanium metal was deposited on the cathode. Spent electrolyte depleted in potassium fluotitanate and sodium chloride content, and containing 30 sodium fluoride and potassium fluoride in an amount stoichiometrically equivalent to the amount of potassium fluotitanate electrolytically decomposed by the electrolysis, was withdrawn from the electrolytic cell in the vicinity of the cathode.

35 The chlorine gas evolved from the electrolytic cell was burned with hydrogen gas to form hydrogen chloride which, in turn, was absorbed in sufficient water to form a solution of hydrochloric acid. The spent electrolyte containing potassium fluoride and sodium fluoride as its 40 essential components was allowed to cool to ambient temperature. The cooled spent electrolyte and the aqueous solution of hydrochloric acid was then introduced into a reaction vessel maintained at about the boiling point of water by means of steam coils. Also present in the reaction vessel was a quantity of titanium dioxide 45 sufficient to react with the potassium fluoride and sodium fluoride content of the spent electrolyte to form an equivalent amount of potassium fluotitanate, and sufficient water to retain the products of the reaction in solution.

The spent electrolyte, hydrochloric acid, and titanium dioxide in the hot aqueous medium reacted together to 50 form soluble reaction products. The aqueous solution from the reaction vessel was then introduced into the third effect of a triple effect evaporator, the temperature of the liquor in which was maintained at about 50° C. 55 Vapor evaporated from the liquor in the third effect was withdrawn therefrom by a conventional condenser and vacuum pump arrangement. Concentrated liquor from the third effect was introduced into a separator from which potassium fluotitanate crystallized from the solution. 60 The crystallized potassium fluotitanate was then dried preparatory to introducing this material into the fused salt electrolyte contained in the electrolytic cell.

65 Concentrated liquor from the separator of the third effect was introduced into the second effect in which the liquor was maintained at a temperature of about 90° C. Vapor evaporated from the liquor in the second effect was introduced into the steam chest of the third effect as in conventional practice. The concentrated liquor from the second effect containing crystals of sodium chloride was introduced into a separator from whence the crystallized sodium chloride was removed. The sodium chloride was then dried preparatory to introducing this material into the fused salt electrolyte.

The concentrated liquor from the separator of the second effect was introduced into the first effect which operated at a temperature of about 130° C. Vapor evaporated from the liquor in the first effect was introduced into the steam chest of the second effect to heat the liquor therein. Concentrated liquor from the first effect was introduced into the second effect for further concentration of its salt content.

The potassium fluotitanate obtained from the dryer associated with the separator of the third effect and the sodium chloride obtained from the dryer associated with the separator of the second effect were introduced into the fused salt electrolyte being electrolyzed in the electrolytic cell. The amount of titanium which reacted with the potassium fluoride and sodium fluoride content of the spent electrolyte and with the hydrochloric acid was stoichiometrically equivalent to the amount of potassium fluotitanate electrolytically decomposed by the cell to form titanium metal, chlorine gas and spent electrolyte containing potassium fluoride and sodium fluoride.

Typical spent electrolytes resulting from the electrolysis of an alkali metal fluozirconate-alkali metal chloride bath are set forth in a copending application Serial No. 279,471, now Patent 2,687,340. Expressed as ions three such baths are disclosed as follows:

| I                     | II                  | III                |
|-----------------------|---------------------|--------------------|
| 33.2% Na <sup>+</sup> | 53% Na <sup>+</sup> | 66% K <sup>+</sup> |
| 24.8% K <sup>+</sup>  | 41% F <sup>-</sup>  | 30% F <sup>-</sup> |
| 36.4% F <sup>-</sup>  | 6% Cl <sup>-</sup>  | 4% Cl <sup>-</sup> |
| 5.6% Cl <sup>-</sup>  |                     |                    |

Each of these spent electrolytes may be readily regenerated in accordance with our invention by reacting the spent electrolyte with HCl obtained from all of the cell chlorine and with a titanium or, in this instance, a zirconium compound such as the carbide, carbonate or oxide, the latter being present in an amount sufficient to provide the amount of zirconium necessary to form the double fluoride of zirconium and an alkali metal when combined with the fluorine content of the spent electrolyte.

It will be seen, accordingly, that the process of our invention makes possible the continuous production of titanium or zirconium metal by electrolysis of a fused salt bath comprising an alkali metal-titanium or zirconium double fluoride and an alkali metal chloride and that our process makes it possible to regenerate these bath components from the spent electrolyte without the introduction into the process, either as the titaniferous or zirconiferous source material or as the digesting medium for these materials, of any elements which would tend to accumulate in the cyclic operation which characterizes our process. The only extraneous elements introduced into our process are limited to chlorine, oxygen, carbon and hydrogen, and each of these elements ultimately is consumed in the formation of water or a permanent gas which is readily discharged from the process as outlined hereinbefore. The relatively expensive components of the system, particularly the fluorine and alkali metal components, are thus continuously recycled. The commercial appeal of the electrolytic production of titanium and zirconium metal is thereby enhanced and an integrated process is obtained in which only relatively simple forms of raw materials are required for the continuous production of these metals in a state of high purity.

We claim:

1. In the production of a metal of the group consisting of titanium and zirconium wherein a fused salt bath consisting essentially of an alkali metal chloride and a double fluoride of an alkali metal and a metal of the group consisting of titanium and zirconium in electrolytically decomposed with (1) the resulting production of an electrodeposit of said metal on a cathode, (2) the evolution of

70  
75

chlorine gas at an anode and (3) the formation of a spent electrolyte consisting essentially of at least one alkali metal fluoride; the improvement which comprises regenerating material suitable for reuse as the fused salt bath in the aforesaid electrolytic process from said evolved chlorine and said spent electrolyte as follows: reacting the evolved chlorine with hydrogen to form hydrogen chloride; heating to up to about 100° C. an aqueous solution of the spent electrolyte and said hydrogen chloride and a compound of said metal from the group consisting of compounds of the said metal and at least one element of the group consisting of oxygen and carbon in which the relative amounts of alkali metal, halogen and metal values present are substantially the stoichiometric amounts necessary to produce the desired double fluoride of an alkali metal and the metal of the group consisting of titanium and zirconium and recovering said double fluoride and said alkali chloride produced in said heated solution for reuse in a repetition of the electrolysis.

2. In the production of a metal of the group consisting of titanium and zirconium wherein a fused salt bath consisting essentially of an alkali metal chloride and a double fluoride of an alkali metal and a metal of the group consisting of titanium and zirconium is electrolytically decomposed with (1) the resulting production of an electrodeposit of said metal on a cathode, (2) the evolution of chlorine gas at an anode and (3) the formation of a spent electrolyte consisting essentially of at least one alkali metal fluoride; the improvement which comprises regenerating material suitable for reuse as the fused salt bath in the aforesaid electrolytic process from said evolved chlorine and said spent electrolyte as follows: reacting the evolved chlorine with hydrogen to form hydrogen chloride; heating to up to about 100° C., an aqueous solution of the spent electrolyte and said hydrogen chloride and an oxide of said metal in which the relative amounts of alkali metal, halogen and metal values present are substantially in the stoichiometric proportions necessary for the formation of a double fluoride of said metal and an alkali metal chloride and recovering said double fluoride and said alkali chloride from said heated aqueous solution for reuse in a repetition of the electrolysis.

3. In the production of a metal of the group consisting of titanium and zirconium wherein a fused salt bath consisting essentially of sodium chloride and a double fluoride of potassium and a metal of the group consisting of titanium and zirconium is electrolytically decomposed with (1) the resulting production of the electrodeposit of said metal on a cathode, (2) the evolution of chlorine gas at an anode and (3) the formation of a spent electrolyte consisting essentially of alkali metal and halide ions; the improvement which comprises regenerating material suitable for reuse as the fused salt bath in the aforesaid electrolytic process from said evolved chlorine and said spent electrolyte as follows: reacting the evolved chlorine with hydrogen to form hydrogen chloride; heating to up to about 100° C., an aqueous solution of the spent electrolyte and said hydrogen chloride and an oxide of said metal in which the relative amounts of alkali metal, halogen and metal values present are substantially in the stoichiometric proportions necessary for the formation of a double fluoride of said metal and an alkali metal chloride and recovering said double fluoride and said alkali chloride for reuse in a repetition of the electrolysis.

4. In the production of a metal of the group consisting of titanium and zirconium wherein a fused salt bath consisting essentially of an alkali metal chloride and a double fluoride of an alkali metal and a metal of the group consisting of titanium and zirconium is electrolytically decomposed with (1) the resulting production of an electrodeposit of said metal on a cathode, (2) the evolution of chlorine gas at an anode and (3) the formation of a spent electrolyte consisting essentially of at least one

alkali metal fluoride; the improvement which comprises regenerating material suitable for reuse as the fused salt bath in the aforesaid electrolytic process from said evolved chlorine with hydrogen to form hydrogen chloride; heating to up to about 100° C., an aqueous solution of the spent electrolyte and said hydrogen chloride and a compound of said metal from the group consisting of compounds of said metal and at least one of the following carbon and oxygen, in which the relative amounts of alkali metal, halogen and metal of the group consisting of titanium and zirconium present are substantially the stoichiometric proportions necessary for the formation of an aqueous medium containing a double fluoride of said metal and an alkali metal and an alkali metal chloride; charging the aqueous medium to the third effect of a 15 triple effect evaporator and therein concentrating the aqueous medium to an extent sufficient to promote crystallization therefrom of the double fluoride; crystallizing the double fluoride, recovering the crystallized double fluoride from the effluent from the third effect of the evaporator; delivering the remaining aqueous medium to the

second and first effects of the evaporator; further concentrating the aqueous medium to an extent sufficient to promote crystallization therefrom of the alkali metal chloride; crystallizing the alkali metal chloride recovering 5 said crystallized alkali metal chloride, and using the recovered double fluoride and alkali metal chloride as the components of said fused salt bath in a repetition of the electrolysis.

## References Cited in the file of this patent

## UNITED STATES PATENTS

|           |          |               |
|-----------|----------|---------------|
| 1,801,661 | Collings | Apr. 21, 1931 |
| 2,144,339 | Laist    | Jan. 17, 1939 |
| 2,687,340 | Wainer   | Aug. 24, 1954 |

## FOREIGN PATENTS

|         |               |               |
|---------|---------------|---------------|
| 574,832 | Great Britain | Jan. 22, 1946 |
|---------|---------------|---------------|

## OTHER REFERENCES

- 20 "Journal of Applied Chemistry (U. S. S. R.)," vol. 13, 1940, pages 51 thru 55; paper by Sklarenko et al.